

H. C. BAINES,  
TREATMENT OF IRON OR STEEL OR OTHER ARTICLES.  
APPLICATION FILED AUG. 10, 1916.

1,303,627.

Patented May 13, 1919.



INVENTOR,  
Henry C. Baines

118 Hull, Smith, Brock West,  
ATTYS.

# UNITED STATES PATENT OFFICE.

HENRY C. BAINES, OF SPRINGFIELD, MASSACHUSETTS, ASSIGNOR, BY MESNE ASSIGNMENTS, TO THE CLEVELAND METAL PRODUCTS COMPANY, OF CLEVELAND, OHIO, A CORPORATION OF OHIO.

## TREATMENT OF IRON OR STEEL OR OTHER ARTICLES.

1,303,627.

Specification of Letters Patent. Patented May 13, 1919.

Application filed August 10, 1916. Serial No. 114,196.

To all whom it may concern:

Be it known that I, HENRY C. BAINES, a subject of the King of England, residing at Springfield, Mass., in the county of Hampden and State of Massachusetts, U. S. A., have invented certain new and useful Improvements in the Treatment of Iron or Steel or other Articles, of which the following is a specification.

10 This invention relates to the treatment of iron or steel or articles having a surface of iron or steel.

The treatment referred to consists in effecting a deposit of phosphate of iron, or a deposit consisting of a mixture of normal ferric and ferrous phosphates of iron, upon the surfaces of the articles; and the general objects of the invention are to accomplish this result in a much shorter time than that 20 heretofore required, to insure a relatively deep penetration of the deposit into the iron of which the articles are composed or with which they are surfaced, to prevent the evaporation of the solution employed for 25 coating the said articles, to retain the liberated hydrogen (thereby insuring a more vigorous reaction than has hitherto been attained), to protect the solution and its contents from oxygen such as contained in the 30 atmosphere (thereby preserving the solution in working condition), and to increase the solubility of the compounds employed in the reaction. A further object of the invention is to employ in connection with the 35 rust-proofing treatment a controlling or regulating agent, such, for instance, as iron filings, which will coöperate in the production of a deposit or coating of normal ferric and ferrous phosphates of iron.

40 In realizing my invention, the articles to be treated are subjected to the action of a dilute solution of phosphoric acid (preferably in the presence of iron filings or powder) in a sealed vessel and the vessel 45 and the contents are heated to a temperature which is generally above that required to bring the solution to the boiling point under ordinary atmospheric conditions. In practice, I generally heat the vessel and its con-

tents to a temperature sufficient to develop 50 therewithin a pressure of several atmospheres; in fact, the pressure may be as high as twenty-five atmospheres, depending upon the speed with which it is desired to accomplish the rust-proofing and the depth of 55 penetration of the phosphate deposit.

A solution or compound which gives satisfactory results is as follows:

|                               |                   |
|-------------------------------|-------------------|
| Iron in the form of filings   | 60                |
| or powder                     | 2 ounces.         |
| Phosphoric acid, concentrated | 4 fluid ounces.   |
| Water                         | 160 fluid ounces. |

The above solution or a dilute solution of 65 ordinary phosphoric acid and water in proper proportions, together with the iron filings or powder or other controlling or regulating agent, may be placed in a stationary, rotatable or other enameled or 70 other sealed vessel and heated to the desired temperature. The articles to be treated, having been previously cleaned in any suitable manner are then suspended in the solution. The heat incident to the boiling operation is confined within the vessel, preventing evaporation, enabling the subjecting of the articles to such temperatures as may be desired or necessary, and insuring 75 such pressure within the vessel as to cause 80 a greater degree of penetration of the solution and coating into the metal than is accomplished by the processes of treatment now in use. By virtue of the deeper penetration of the solution into the metal, I provide 85 an efficient and durable coating of the nature hereinbefore stated. The articles thus treated, are then withdrawn, dried and oiled for use.

The coating or deposit formed upon the 90 articles may be strengthened or thickened, according to the proportions of the ingredients. Should the coating be too thick, the excess may be removed by subjecting the coated article to the action of cold water. 95 If it be desired to vary the tone or color of the protective coating, the articles may be subjected to a suitable solution for the pur-

pose. A suitable solution for this purpose is a solution of a chemical or chemicals that will react with the coating to alter the chemical composition of such coating and 5 the color and texture thereof. Solutions of sulfids, copper salts, tannin, etc., may be employed for this purpose.

The particular means for heating the solution is immaterial, for any suitable heating 10 means may be employed. If desired, an electric current may be passed through the dilute solution of ordinary phosphoric acid with or without the aforesaid controlling or regulating agent.

15 If desired, the coating solution may consist of liquid concentrated phosphoric acid; manganese dioxid and water in suitable proportions; or zinc, phosphoric acid and water in suitable proportions may be employed; or other suitable compounds or 20 solutions may be employed.

In the drawing there is shown a vertical sectional view through a vessel containing a solution of the character described and showing 25 the connections whereby a current of electricity may be passed through the solution, part of the means for supplying the current being illustrated diagrammatically. In the said drawing, 1 denotes the body of the 30 receptacle, which will be of conducting material, said body being provided with a flange 2 at the top to which the cover 3 may be secured by means of swinging bolts 4 pivoted in recesses within said flange and having 35 wing nuts 5 for drawing the cover securely to its seat. A gasket 6 is shown as interposed between the cover and the flange.

The vessel is shown as provided with inwardly projecting ledges 7 forming seats for 40 a rod 8 of conducting material, the ends of the rod resting upon insulating material 9. 10 denotes any convenient source of electric energy, 11 a conductor leading therefrom to the wall of the tank and being electrically 45 connected thereto, as indicated at 1<sup>a</sup>. Opposite the connection 1<sup>a</sup> the tank wall is provided with a bushing 12 of insulating material through which the conductor 11<sup>a</sup> extends, said conductor leading to the source 50 of electrical energy 10. An ordinary type of switch is indicated at 11<sup>b</sup>. The solution and regulating or controlling agent having been introduced into the tank, the articles to be treated (indicated at 13, 14 and 15) are 55 suspended in the solution from the rod 8 and the cover applied so as to seal the vessel or tank. The tank or vessel is then heated to the desired temperature and a current of electricity may be passed therethrough by 60 closing the switch 11<sup>b</sup>.

What is claimed is:—

1. The treatment of iron or steel for the purpose of preventing the oxidation or rusting thereof which comprises subjecting the

same to the action of a solution of phosphoric acid under pressure greater than that of the atmosphere.

2. The treatment of iron or steel for the purpose of preventing the oxidation or rusting thereof which comprises subjecting the 70 same to the action of a phosphate solution under pressure greater than that of the atmosphere.

3. The treatment of iron or steel for the purpose of preventing the oxidation or rusting 75 thereof which comprises subjecting the same to the action of a phosphate solution with the substantial exclusion of oxygen.

4. The treatment of iron or steel for the purpose of preventing the oxidation or rusting 80 thereof which comprises subjecting the same to the action of a solution of phosphoric acid with the practical exclusion of oxygen.

5. The treatment of iron or steel which comprises subjecting the same to a solution 85 of phosphoric acid and a controlling or regulating agent in a sealed vessel the temperature whereof is in excess of that of the normal boiling point of such solution.

6. The treatment of iron or steel which 90 comprises subjecting the same to a phosphate solution in a sealed vessel whereby oxygen is substantially excluded and hydrogen retained.

7. The treatment of iron or steel which 95 comprises subjecting the same to a solution of phosphoric acid in a sealed vessel heated to a temperature whereby the pressure within such vessel will be in excess of that of the atmosphere and passing an electric current 100 through the solution and the articles to be coated.

8. The treatment of iron or steel which comprises subjecting the same to a phosphate solution in a sealed vessel and subjecting the 105 coating thus produced to a solution capable of chemically combining with the coating to alter the color or texture thereof.

9. The treatment of iron or steel which comprises subjecting the same to a phosphate 110 solution under pressure.

10. The treatment of iron or steel which comprises subjecting the same to a phosphate solution and subjecting the coating thus produced to a solution capable of chemically 115 combining with the coating to alter the color or texture thereof.

11. The treatment of iron or steel which comprises subjecting the same to a phosphate solution under pressure and subjecting the 120 coating thus produced to a solution capable of chemically combining with the coating to alter the color or texture thereof.

12. The treatment of iron or steel which comprises subjecting the same to a phosphate 125 solution in the presence of the metallic base of said solution, the aforesaid operations being carried out in a sealed vessel heated to

a temperature sufficient to produce a pressure within said vessel greater than that of the atmosphere.

13. The treatment of iron or steel which 5 comprises subjecting the same to the action of a phosphate solution under pressure greater than that of the atmosphere, passing an electric current through such solution and the article or articles to be coated, and sub-  
10 jecting the article or articles to a solution

capable of chemically combining with the coating thereon to alter the color or texture thereof.

In testimony whereof I affix my signature in the presence of two witnesses.

HENRY C. BAINES.

Witnesses:

R. BAINES,  
AMOS K. HOBBY.